

1

3,700,455

COLOR PHOTOGRAPH CONTAINING FADE-PREVENTING AGENTS

Hidehiko Ishikawa, Mikio Sato, and Syun Takada, Odawara, Japan, assignors to Konishiroku Photo Industry Co., Ltd., Tokyo, Japan

No Drawing. Filed Aug. 31, 1970, Ser. No. 68,534  
Claims priority, application Japan, Sept. 5, 1969,

44/69,945

Int. Cl. G03c 1/40, 7/00, 1/84  
U.S. Cl. 96—100 4 Claims

ABSTRACT OF THE DISCLOSURE

A compound of the formula,



wherein R<sub>1</sub>, R<sub>2</sub>, R<sub>3</sub> and R<sub>4</sub> are individually a straight chain or branched-chain hydrocarbon radical having 1 to 18 carbon atoms, the total sum of carbon atoms of said R<sub>1</sub>, R<sub>2</sub>, R<sub>3</sub> and R<sub>4</sub> being less than 32; and X is —S—, —O—, —SO<sub>2</sub> or



where n is an integer of 0 to 3, and R<sub>5</sub> is a hydrogen atom or a lower alkyl group, and a color image-forming dye are incorporated into a silver halide photographic composition. When developed, a color image having improved light fastness is obtained. An ultraviolet ray absorbing agent and/or a color coupler may be incorporated into the composition.

The present invention relates to a color photograph bearing a color image comprising an azomethine, indoaniline or the like dye together with a phenol derivative as a fading-preventing agent.

It is well known that a color photograph is obtained by subjecting a light-sensitive silver halide color photographic material to color development according to the oxidation condensation reaction of primary aromatic amino compound with a coupler, thereby forming a color image comprising an azomethine, indoaniline, indophenol or the like dye. In this case, subtractive color photography is employed for reproduction of the color image, and cyan, magenta and yellow dyes are formed by the color development, in general. Ordinarily, the cyan dye is formed from a phenol or naphthol type coupler, the magenta dye from a pyrazolone type coupler, and the yellow dye from an acylacetamide type coupler. These couplers are added to developers or have previously been incorporated into silver halide photographic emulsions.

However, it is also well known that a color image formed according to such color development process as mentioned above is not satisfactory in fastness resistance chiefly to ultraviolet rays or visible light (hereinafter referred to as "light fastness"), and is faded with relative ease when irradiated with ultraviolet rays or visible light. In order to overcome the above-mentioned drawbacks, there have heretofore been studied many processes for improving a color image in light fastness by incorporating an ultraviolet ray-absorbing agent into a light-sensitive silver halide color photographic material, thereby decreasing the dose of ultraviolet rays irradiated to the

2

resulting color image. However, in order to impart satisfactory light fastness to a color image by use of an ultraviolet ray-absorbing agent, a large amount of said agent is required, thereby the color image is greatly stained due to coloration of the ultraviolet ray-absorbing agent itself. Further, the use of an ultraviolet ray-absorbing agent is not effective at all for prevention of the fading of color image due to visible light, and thus the improvement in light fastness of color image by use of an ultraviolet ray-absorbing agent has a limit.

In view of such actual state as mentioned above, we made studies for years in order to improve the light-fastness of color images formed by color development of light-sensitive silver halide color photographic materials. As the result, it has been found that the light fastness of a developed color image is greatly improved by making present, together with a dye in the developed color image, a bisphenol derivative of the general formula,



wherein R<sub>1</sub>, R<sub>2</sub>, R<sub>3</sub> and R<sub>4</sub> are individually a straight chain or branched chain hydrocarbon radical having 1 to 18 carbon atoms, the total sum of carbon atoms of said R<sub>1</sub>, R<sub>2</sub>, R<sub>3</sub> and R<sub>4</sub> being less than 32; and X is —S—, —O—, —SO<sub>2</sub> or



where n is an integer of 0 to 3; and R<sub>5</sub> is hydrogen atom or a lower alkyl group.

The above-mentioned fading-preventing agent employed in the present invention is used for the improvement in light fastness of cyan, magenta and yellow color images formed by color development. Cyan, magenta and yellow couplers to be used for the formation of these color images are not limited, and may be any of such types that they are alkali-soluble and alkali solutions thereof are incorporated into silver halide photographic emulsions, and that they are dissolved in a high boiling organic solvent to give a solution which can be dispersed in an aqueous gelatine solution or added to silver halide photographic emulsions.

The fading-preventing agent employed in the present invention may be incorporated into any or all of the layers of a light-sensitive silver halide photographic materials, i.e. photographic emulsion layers in which cyan, magenta and yellow dyes will be formed by color development. Further, when applied to a transfer diffusion method, the fading-preventing agent may be incorporated not only into such photographic emulsion layers as mentioned above but also into receptive layers. That is, it is sufficient that the fading-preventing agent is made present together with any or all of dyes forming the color image of a finally obtained photograph.

The fading-preventing agent used in the present invention is hardly water-soluble, and it is dissolved in a low boiling organic solvent such as methyl acetate, ethyl acetate, carbon tetrachloride, chloroform, methanol, ethan, n-butanol, dioxane, acetone, benzene, dimethylformamide or dimethyl sulfoxide, a high boiling solvent such tricresyl phosphate, di-n-butyl phthalate or ethyl N,N-diphenyl carbamate, or a mixed solvent comprising said low and high boiling solvents. The resulting solution is charged into a protective colloid solution, dispersed by means of a colloid mill or a homogenizer and then added

to, for example, a silver halide photographic emulsion containing a coupler. Depending on the type of the coupler, the fading-preventing agent and the coupler may be dissolved in an organic solvent and then added to an aqueous gelatine solution or the like.

Examples of the fading-preventing agent used in the present invention are as shown below, but these are, of course, not limitative.

(1)



(2)



(3)



(4)



(5)



(6)



(7)



The amount of the fading-preventing agent to be added varies depending on the kind of said agent and the coupler employed and on the kind of the layer to which the agent is applied, but is usually within the range from 1 to 100% by weight based on the weight of the coupler. A silver halide photographic emulsion containing the fading-preventing agent and a coupler is coated on a support such as baryta paper or film base to form a photographic emulsion layer. Into this photographic emulsion layer, or a lower or upper layer thereof, may be incorporated an ultraviolet ray-absorbing agent. Thus the fading-preventing agent of the present invention can be used in combination with the ultraviolet ray-absorbing agent, whereby the light fastness of the resulting color image can be enhanced. Examples of the ultraviolet ray-

absorbing agent to be used in the above case are benzophenone, acrylonitrile, thiazolidone, benzotriazole, stilbene, oxazole, thiazole and imidazole type compounds, though these are, of course, not limitative.

When, as mentioned above, dyes forming the color image of a color photograph are made present together with a fading-preventing agent represented by the aforesaid general formula, the resulting developed color image is markedly improved in fastness to ultraviolet rays and visible light, as will be clear from the examples set forth later. Further, all the fading-preventing agents used in the present invention are substantially colorless and hence do not stain the resulting color images.

The incorporation of the fading-preventing agent does not bring about any injury in the color development, and even when it is made present together with a dye formed by color development, no change in hue is observed. Moreover, the fading-preventing agent has no detrimental interactions with other photographic additives.

The present invention is illustrated below with reference to examples.

#### EXAMPLE 1

2 g. of the exemplified compound (4) was dissolved in a mixed solution of 1 g. of tricresyl phosphate and 4 g. of ethyl acetate. The resulting solution was added to 40 cc. of a 5% aqueous gelatine solution containing saponin and then dispersed by means of a homogenizer. The whole amount of the resulting dispersion was added to 400 cc. of a silver chlorobromide emulsion containing 10 g. of sodium 1-hydroxy-N-octadecyl-2-naphthamide-4-sulfonate (coupler). Thereafter, the emulsion was coated on a baryta paper and then dried to prepare a sample of the present invention.

For comparison, a control sample was prepared in the same manner as above, except that the compound (4) was not used.

The sample of the present invention and the control sample were individually exposed to white light, subjected to color development, stopping, fixing, bleaching, water-washing and drying, and exposed for 5, 10 and 20 hours by means of a Xenon fade meter to calculate the percentage ( $D/D_0 \times 100$ ) of the density after exposure (D) to the density before exposure ( $D_0$ ). The results were as shown in Table 1.

TABLE I

| Sample                               | $D/D_0 \times 100$ |    |    |
|--------------------------------------|--------------------|----|----|
| Control sample.....                  | 82                 | 65 | 41 |
| Sample of the present invention..... | 94                 | 88 | 76 |
| Exposure time (hrs.).....            | 5                  | 10 | 20 |

NOTE.— $D_0 = 1.0$ .

As is clear from the results shown in Table 1, the light fastness of the sample of the present invention is greatly improved.

#### EXAMPLE 2

A mixture comprising 8.0 g. of the cyan coupler 2-(p-tert-amylphenoxy-p-benzoyl)-amino-4-chloro-5-methylphenol, 3.0 g. of the exemplified compound (2) and 3.0 g. of the ultraviolet ray-absorbing agent 2-(2'-hydroxy-3',5-di-tert-butylphenyl)-benzotriazole was dissolved in a mixed solution of 8 g. of tricresyl phosphate and 20 g. of ethyl acetate. The resulting solution was added to 200 cc. of a 5% aqueous gelatine solution containing saponin and then dispersed by means of a homogenizer. Subsequently, the resulting dispersion was added to 400 cc. of a red-sensitive silver iodobromide emulsion, which was then coated on a film base, followed by drying, to prepare a sample (I) of the present invention.

Further, a control sample, a sample (II), and a sample (III) were prepared in the same manner as above, except that there were not used, respectively, both the exemplified compound (2) and the ultraviolet ray-absorbing agent.

The samples (I) to (III) and the control sample were individually exposed to white light, subjected to color

development, stopping, fixing, bleaching washing and drying, and then exposed for 10, 20 and 40 hours by means of a xenon fade meter to measure the density variation of the samples in the same manner as in Example 1. The results were as shown in Table 2.

TABLE 2

| Sample               | D/Do×100 |    |    |
|----------------------|----------|----|----|
| Control sample       | 85       | 71 | 54 |
| Sample:              |          |    | 10 |
| I                    | 100      | 98 | 95 |
| II                   | 94       | 87 | 80 |
| III                  | 97       | 92 | 90 |
| Exposure time (hrs.) | 10       | 20 | 40 |

NOTE.—Do=1.0.

From the results of Table 2, it is evident that the samples (I) and (III) of the present invention show excellent light fastness, which is further enhanced by use of the exemplified compound (2) in combination with the ultraviolet ray-absorbing agent.

### EXAMPLE 3

A mixture comprising 10 g. of the magenta coupler 1-(2,4-dimethyl - 6 - chlorophenyl-7,3-{3-[ $\alpha$ -(3-penta-decylphenoxy)butylamide]benzamide}-5-pyrazolone and 4 g. of the exemplified compound (1) was dissolved in a mixed solution of 5 g. of dibutyl phthalate and 20 g. of ethyl acetate. The resulting solution was added to 200 cc. of a 5% aqueous gelatine solution containing saponin and then dispersed by means of a homogenizer. Subsequently, the dispersion was added to 350 cc. of a green-sensitized silver chlorobromide emulsion, which was then coated on a baryta paper.

On the other hand, 7 g. of the same ultraviolet ray-absorbing agent as in Example 2 was dissolved in a solution of 10 g. of tricresyl phosphate in 20 g. of ethyl acetate. The resulting solution was added to 300 cc. of a 10% aqueous gelatine solution containing saponin and then dispersed by means of a homogenizer. The thus obtained dispersion was coated on the aforesaid silver chlorobromide emulsion layer so that the amount of the ultraviolet ray-absorbing agent became 7 mg. per 100 cm.<sup>2</sup>, followed by drying, to prepare a sample (I).

Further, samples (II) and (III) and a control sample were prepared in the same manner as above, except that there were not used, respectively, the ultraviolet ray-absorbing agent, the exemplified compound (1), and both the ultraviolet ray-absorbing agent and the exemplified compound (1).

The thus prepared samples (I) to (III) and the control sample were individually subjected to the same photographic treatments as in Example 1, and then exposed for 5, 10 and 20 hours by means of a xenon fade meter to calculate the density variation of the samples in the same manner as in Example 1. The results were as shown in Table 3.

TABLE 3

| Sample               | D/Do×100 |     |    |
|----------------------|----------|-----|----|
| Control sample       | 70       | 53  | 38 |
| Sample:              |          |     |    |
| I                    | 100      | 100 | 96 |
| II                   | 93       | 96  | 87 |
| III                  | 83       | 66  | 50 |
| Exposure time (hrs.) | 5        | 10  | 20 |

NOTE.—Do=1.0.

From the results of Table 3, it is clear that the samples (I) and (II) of the present invention are excellent in light fastness.

What we claim is:

1. A color composition which upon development produces a color image having improved light fastness, said composition comprising

(a) a silver halide photographic emulsion

(b) a compound of the formula,



wherein R<sub>1</sub>, R<sub>2</sub>, R<sub>3</sub> and R<sub>4</sub> are individually a straight chain or branched-chain hydrocarbon radical having 1 to 18 carbon atoms, the total sum of carbon atoms of said R<sub>1</sub>, R<sub>2</sub>, R<sub>3</sub> and R<sub>4</sub> being less than 32, and X is

—S—, —O—, —SO<sub>2</sub> or



where n is an integer of 0 to 3 and R<sub>5</sub> is a hydrogen atom or a lower alkyl group; and

(c) a color coupler of the phenol, naphthol, pyrazolone or acylacetamide type.

2. The composition as claimed in claim 1, further containing an ultraviolet ray-absorbing agent.

3. The composition as claimed in claim 1, wherein said compound is present in an amount of from 1-100% by weight based on the weight of the coupler.

4. The composition as claimed in claim 2, wherein said agent is a benzophenone, acrylonitrile, thiazolidine, benzotriazole, stilbene, oxazole, thiazole or imidazole type compound.

### References Cited

#### UNITED STATES PATENTS

|           |        |                    |       |
|-----------|--------|--------------------|-------|
| 2,688,625 | 9/1954 | Bell et al. -----  | 96—56 |
| 2,735,765 | 2/1956 | Loria et al. ----- | 96—56 |
| 3,271,156 | 9/1966 | Sawdye -----       | 96—56 |

55 J. TRAVIS BROWN, Primary Examiner

U.S. CL. X.R.

96—55, 56, 56.5, 84